

[54] THIN-FILM FIELD-EMISSION ELECTRON SOURCE AND A METHOD FOR MANUFACTURING THE SAME

3,970,887 7/1976 Smith et al. .... 313/309

[75] Inventors: **Isamu Yuito, Hachioji; Kikuji Sato, Kokubunji; Mikio Hirano, Ohme**, all of Japan

Primary Examiner—Saxfield Chatmon, Jr.  
Attorney, Agent, or Firm—Craig & Antonelli

[73] Assignee: **Hitachi, Ltd., Japan**

[57] **ABSTRACT**

[22] Filed: **Aug. 18, 1975**

A thin-film field-emission electron source having an emitter within a minute cavity in a conductive substrate, an insulating layer covering the surface of the substrate except for the portion of the cavity, and a first anode layer on the insulating layer, wherein the substrate and the emitter are comprised as one body, and the insulating layer and the first anode layer overhang the cavity, except directly over the emitter.

[21] Appl. No.: **605,603**

This electron source may be manufactured by the method comprising the steps of i) forming a sandwich structure of the substrate-insulating layer-first anode layer, ii) forming a closed loop opening at a predetermined position on the surface of the first anode layer, iii) etching the insulating layer with the use of the first anode layer as a mask and iv) forming an emitter and a cavity by etching the substrate with the use of the insulating layer as a mask.

[30] **Foreign Application Priority Data**

Aug. 16, 1974 Japan ..... 49-93297

This thin-film field-emission electron source can be manufactured very readily and has good insulation between the emitter and the first anode layer.

[52] U.S. Cl. .... **313/309; 29/580; 313/336; 313/351**

**19 Claims, 21 Drawing Figures**

[51] Int. Cl.<sup>2</sup> ..... **H01J 1/02**

[58] Field of Search ..... **313/309, 336, 351; 156/3, 17, 11; 29/580**

[56] **References Cited**

UNITED STATES PATENTS

|           |         |                       |           |
|-----------|---------|-----------------------|-----------|
| 3,453,478 | 7/1969  | Shoulders et al. .... | 313/336 X |
| 3,500,102 | 3/1970  | Crost et al. ....     | 313/309 X |
| 3,665,241 | 5/1972  | Spindt et al. ....    | 313/309   |
| 3,671,798 | 6/1972  | Lees ....             | 313/309   |
| 3,755,704 | 8/1973  | Spindt et al. ....    | 313/309   |
| 3,814,968 | 6/1974  | Nathanson et al. .... | 313/309   |
| 3,855,499 | 12/1974 | Yamada et al. ....    | 313/336   |
| 3,921,022 | 11/1975 | Levine ....           | 313/309   |



FIG. 1 PRIOR ART



FIG. 2a PRIOR ART



FIG. 2b PRIOR ART



FIG. 2c PRIOR ART



FIG. 2d PRIOR ART



FIG. 3a PRIOR ART



FIG. 3b PRIOR ART



FIG. 3c PRIOR ART



FIG. 3d PRIOR ART



FIG. 3e PRIOR ART



FIG. 4a



FIG. 4b



FIG. 4c



FIG. 4d



FIG. 5



FIG. 6a



FIG. 6b



FIG. 6c



FIG. 6d



FIG. 7a



FIG. 7b



THIN-FILM FIELD-EMISSION ELECTRON  
SOURCE AND A METHOD FOR MANUFACTURING  
THE SAME

BACKGROUND OF THE INVENTION

1. Field of the Invention

The present invention relates to a thin-film field-emission electron source and, more particularly, to a thin-film field-emission electron source which is manufactured by etching layer by layer a sandwich structure of the substrate-insulating layer-first anode layer.

2. Brief Description of the Prior Art

In general, a thin-film field-emission electron source, which will be referred to as MFE (an abridgement of "micro-field-emission type electron source"), has a structure which comprises a first anode 1 and a needle-like emitter 3 which is arranged very closely (for example less than about 10  $\mu\text{m}$ ) to the first anode as is shown in FIG. 1. A MFE is a kind of cold cathode in which the field emission phenomenon is utilized. Electrons are emitted from the emitter, the tip of which is in a strong electric field, by applying a relatively low voltage between the first anode 1 and the emitter 3. Furthermore, there is an insulating layer 2 between the first anode 1 and a substrate 4 which is constructed as one body with the emitter 3.

Heretofore, there have been many problems concerning the formation of the first anode and the emitter in manufacturing MFE's. In that connection, the etching method shown in FIG. 2(a) to FIG. 2(d) will be explained hereunder.

The formation of an insulating layer 2 on a conductive substrate 4 which may also be an insulating substrate having a deposited conductive layer of a predetermined thickness thereon, precedes an etching procedure of the insulating layer 2. This etching is carried out by a well known photoetching technique so as to make the insulating layer form a suitable pattern according to the desired shape of the emitter produced hereafter, for example a circlelike insulating layer on the substrate as is shown in FIG. 2(b). FIG. 2(a) illustrates the double layer of the substrate 4 and the insulating layer 2 produced in the former step. The conductive substrate 4 is then etched with the use of the circlelike insulating layer as a mask. The etching phenomenon thereby advances simultaneously in a direction perpendicular as well as parallel to the face of the substrate, and the portion under the circlelike insulating layer is etched as illustrated in FIG. 2(c). Therefore, an emitter having a sharp tip can be formed. FIG. 2(d) illustrates the completely formed emitter with substrate. However, there is no first anode formed close to the emitter, which is necessary in order to act as a MFE. Accordingly, it is necessary to provide a first anode near the emitter. This procedure has the great disadvantage that the alignment of the first anode with the emitter is very difficult in practice although it can be obtained theoretically.

Another previous method for manufacturing MFE's is illustrated in FIG. 3(a) to FIG. 3(e). This method includes the following steps: i) forming a first conductive layer 5, an insulating layer 2 and a second conductive layer 1 on a substrate 4, in this order, as is shown in FIG. 3(a), ii) etching the second conductive layer 1 so as to form at least one circular opening at a predetermined position, iii) etching the insulating layer 2 employing the second conductive layer having the opening

as a mask, so as to form at least one circular opening reaching the predetermined position on the first conductive layer 5 as is shown in FIG. 3(b), and iv) forming the emitter, having a sharp tip, in the opening. In 5 this method, the shape of the opening in the insulating layer 2 is an inverse truncated cone, and the diameter  $d_1$  of the opening in the second conductive layer 1 is smaller than the upper base diameter of the truncated cone. The second conductive layer 1 overhangs the 10 opening of the insulating layer 2. In the above-mentioned step iv), the emitter 3 is deposited by the simultaneous evaporation method of mask material 8 and emitter material 7. These two materials are evaporated by oblique evaporation and normal evaporation respectively. During the simultaneous evaporation, the substrate 4 is rotated. The mask material 8 is deposited on the second conductive layer 1 forming a gradually closing opening, the diameter of which becomes smaller from  $d_1$  to  $d_2$  as is illustrated in FIG. 3(c). Therefore, 15 the depositing area of the simultaneously evaporated emitter material 7 decreases with decreasing diameter of the mask opening. Finally, the opening of the second conductive layer 1 is closed by the deposited mask material 6 and an emitter with a sharp tip is formed as is shown in FIG. 3(d). Then, the oblique evaporated material 6 which is a mixture of mask material 8 and emitter material 7 is selectively dissolved and removed. 20 As the result, there is obtained a MFE having an emitter 3 with a sharp tip and a first anode 1. FIG. 3(e) shows this resulting MFE. However, this method has many difficulties in that i) the character of the emitter material changes because of the mixing of the mask material with the emitter material by the simultaneous evaporation, ii) selective removal of the mask material 30 layer 6 is necessary and iii) the apparatus for the simultaneous vacuum evaporation of the two materials is very complicated, and so on. Furthermore, MFE's produced according to this method, and having the structure illustrated in FIG. 3(e), have great difficulties in 35 that the surface 2' of the insulating layer is open to dielectric breakdown of the insulation because of frequent contamination of the surface 2' during operation. Indeed, the insulation between the emitter 3 and the first anode 1 depends greatly on the insulating character at the surface 2' of the insulating layer 2.

SUMMARY OF THE INVENTION

The object of the present invention is to overcome the above-mentioned difficulties with the structure and 50 production of prior MFE. Namely, it is an object of the present invention to provide a trouble-free MFE having improved insulation between the emitter and the first anode. Another object of the present invention is to provide a novel method for producing the aforementioned MFE's without difficulty.

To achieve the above-mentioned objects, the thin-film field-emission electron source of the present invention has a needlelike emitter within a minute cavity in a conductive substrate, an insulating layer on the 55 surface of the substrate except for the portion of the cavity, and a first anode layer on the insulating layer, wherein said substrate and said emitter are comprised as one body, and said insulating layer and said first anode layer overhang said cavity around the projection 60 of said emitter except directly over said emitter.

The method of the present invention for producing said electron source comprises the following steps: i) forming an insulating layer on a conductive substrate,

ii) forming a first anode layer made of conductive material on said insulating layer to provide a sandwich structure of the substrate-insulating layer-first anode layer, iii) forming a closed loop opening (i.e. an annular opening) at a predetermined position on said first anode layer by the well known photo-etching technique, wherein said opening reaches to the surface of said insulating layer, iv) etching said insulating layer, employing said first anode layer as a mask to form a closed loop opening (i.e. an annular opening) under the first anode opening provided in step iii), wherein said opening reaches to the surface of said substrate, and v) etching said substrate, employing said insulating layer as a mask to form a cavity and a needlelike emitter which is under the level of said insulating layer and the projection of which is surrounded by said opening of said insulating layer, and to thereby remove portions of said insulating layer and first anode layer which are surrounded by said openings, and to thereby generate a large opening in said insulating layer.

Said substrate may also be made of an insulating plate, such as a sapphire plate, on which a conductive layer is formed. In the case of this composite substrate, said emitter is made from the conductive layer on the insulating plate and is electrically connected thereto. Accordingly, the thickness of said conductive layer must be greater than the height of said emitter.

Suitable materials for the conductive substrate are, for example, Si, W, W alloyed with Th, Mo and so on. It is desirable for the conductive substrate material to have both electric conductivity and a low work function.

Dense and hard insulating materials having appropriate dielectric breakdown voltages and high melting temperatures, such as  $\text{SiO}_2$ ,  $\text{TiO}_2$ ,  $\text{La}_2\text{O}_5$ ,  $\text{Y}_2\text{O}_3$ ,  $\text{Si}_3\text{N}_4$ , AlN, alumina and heat resisting glass, are preferably used for said insulating layer. These insulating materials are provided on the conductive substrate by the well known chemical vapor deposition method, thermal oxydization method or sputtering method. Generally, the thickness of the insulating layer is 0.4  $\mu\text{m}$  to 5  $\mu\text{m}$ . The material and the thickness of said insulating layer must be selected so as to have a dielectric breakdown voltage of higher than 100 V because they relate to the insulation between said emitter and first anode.

The material for said first anode layer must be conductive, and is generally formed by the evaporation method. The desirable thickness of the first anode layer ranges from 0.1  $\mu\text{m}$  to 2  $\mu\text{m}$  in MFE's manufactured according to the aforementioned method. The excessively thick layers have difficulty during the photoetching. In the method shown by FIGS. 6(a) to 6(d) and disclosed later, the desirable range of the first anode layer is from 0.04  $\mu\text{m}$  to 1  $\mu\text{m}$ . In the case of the production method mentioned above, the material of said first anode layer must be determined according to the kind of etchant of said insulating layer and said substrate. For example, if the etchant is hydrofluoric acid aqueous solution, a hydrofluoric acid resisting conductor, for example, Cr, Au, Ni and their alloys are desirable for the material of said first anode material.

Physical etching techniques such as plasma gas etching, ion etching and sputter etching may be used in place of the conventional chemical etching technique for the etching of at least one of said first anode layer, insulating layer, and substrate. An etching method combining these techniques may also be used. How-

ever, in general, only the chemical etching technique is used.

Furthermore, in the method for manufacturing said electron source, electron emissive material layers may be deposited on said first anode layer and said emitter to improve the electron emission of said emitter after the aforesaid step v). The electron emissive material on the first anode layer is not necessary, but it is naturally deposited thereon by the vacuum evaporation step 10 which might be used in such procedures.

The typical material for said electron emissive material is  $\text{LaB}_6$ , but there may also be used for this purpose barium oxide compounds such as  $(\text{Ba},\text{Sr})\text{O}$  and  $(\text{BaO}-\text{SrO}-\text{CaO})$ , calcium oxide compounds such as  $(\text{Ca},\text{Sr})\text{O}$ , boron compounds such as  $\text{LaB}_6$ ,  $\text{CaB}_6$ ,  $\text{SrB}_6$ ,  $\text{BaB}_6$ , and  $\text{CeB}_6$ , lanthanum boride compounds such as  $(\text{La},\text{Sr})\text{B}_6$ ,  $(\text{La},\text{Ba})\text{B}_6$  and  $(\text{La},\text{Eu})\text{B}_6$ , cerium boride compounds such as  $(\text{Ce},\text{Sr})\text{B}_6$ ,  $(\text{Ce},\text{Ba})\text{B}_6$  and  $(\text{Ce},\text{Eu})\text{B}_6$ , praseodymium boride compounds such as  $(\text{Pr},\text{Sr})\text{B}_6$ ,  $(\text{Pr},\text{Ba})\text{B}_6$  and  $(\text{Pr},\text{Eu})\text{B}_6$ , neodymium boride compounds such as  $(\text{Nd},\text{Sr})\text{B}_6$ ,  $(\text{Nd},\text{Ba})\text{B}_6$  and  $(\text{Nd},\text{Eu})\text{B}_6$ , europium boride compounds such as  $(\text{Eu},\text{Sr})\text{B}_6$ ,  $(\text{Eu},\text{Ba})\text{B}_6$ , and so on. These compounds are all hard, and have a low work function and a high melting point.

The above-mentioned electron emissive materials are also used as a conductive layer formed on the insulating plate of the aforementioned composite substrate. The aforesaid conductive substrate materials such as Si, W, 25  $\text{W}$  alloyed with Th, Mo or the like are used for this conductive layer too.

Another method of the present invention for producing said electron source comprises the following steps: i') forming an insulating layer on a conductive substrate, ii') forming a closed loop opening at a predetermined position on said insulating layer by the well known photo-etching technique, wherein said opening reaches to the surface of said substrate, iii') etching said substrate, employing said insulating layer as a mask, to form a cavity and a needlelike emitter which is under the level of said insulating layer and the projection of which is surrounded by said opening of said insulating layer, and thereby removing the portion of said insulating layer which is surrounded by said opening, and iv') depositing an electron emissive material simultaneously on said insulating layer and on said emitter to form a first anode layer on said insulating layer improving the electron emissivity of said emitter. The aforesaid electron emissive materials such as  $\text{LaB}_6$ , 35 barium oxide compounds, calcium oxide compounds and many boride compounds may be used as said electron emissive material in this step (iv'). Other matters described in the foregoing paragraph about the substrate, the insulating layer and the emitter may also be applied to this method. The thickness of the deposited emissive material layer in this step (iv') should preferably range from 0.04  $\mu\text{m}$  to 1.0  $\mu\text{m}$ . Accordingly, in this method, the thickness of the first anode layer is in the range. In both methods, the shape and sharpness of the needlelike emitter and the degree of overhang of the first anode layer and/or the insulating layer over the cavity are suitably controlled by the stirring of the etching solution and by the etching time. It is preferably to have an overhang of greater than 0.5  $\mu\text{m}$ , and more preferable to have one greater than 1  $\mu\text{m}$ . The diameter, or side, of the cavity in the substrate may be 40 2.5 to 10  $\mu\text{m}$ . Furthermore, the diameter, or side, of said large opening of said insulating layer is preferably 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9

in the range from 1.5  $\mu\text{m}$  to 5  $\mu\text{m}$ , and more preferably from 2.5  $\mu\text{m}$  to 3.5  $\mu\text{m}$ . When it is smaller than this, it becomes difficult for gas generated in the cavity during operation to escape. When, on the contrary, it is too large, the gradient of the electric field about the tip of the emitter becomes dull. Both cases are undesirable for a good electron source.

If necessary, there can be formed an electron source comprising plural emitters and first anodes on a single substrate, according to the method of the present invention. Even several thousand emitters and first anodes may be manufactured simultaneously on one substrate, if desired.

The above-mentioned thin-film field-emission electron source according to the present invention has excellent properties and no difficulties in manufacturing. Accordingly, it is very suitable for the cathode of a quick starting Braun tube, a display tube, an electron microscope and so on.

The excellent properties of this MFE, such as good insulation between the emitter and the first anode layer, depend on a structure which has an insulating layer with a long surface between the conductive substrate surrounding the emitter and the first anode layer. Furthermore, a thin-film field-emission electron source having a good alignment of the first anode with the emitter can be readily obtained according to the method of the present invention because of the self-alignment thereof in the etching steps, and/or the electron emissive material depositing step. Accordingly, an extremely high precision of disposition of the first anode and the emitter is obtainable with no resulting inferior products due to excessively short length of the surface of the insulating layers between the conductive substrate and the first anode. The excessively short distance thereof arises from a misalignment of the first anode with the emitter.

Other features and advantages of the invention will be apparent from the following description in connection with the accompanying drawings.

#### BRIEF DESCRIPTION OF THE DRAWINGS

FIG. 1 is a cross-sectional view illustrating the main structure of a MFE.

FIGS. 2a to 2d are diagrammatic illustrations of one previous method for manufacturing a MFE by the etching method.

FIGS. 3a to 3e are diagrammatic illustrations of another previous method for manufacturing a MFE.

FIGS. 4a to 4d are cross-sectional views illustrating the structure of a MFE and the manufacturing steps thereof in an embodiment of the present invention.

FIG. 5 is a diagrammatic illustration which explains a method of depositing material layers, having a low work function, on the MFE obtained by the method shown at FIGS. 4a to 4d.

FIGS. 6a to 6d are cross-sectional views illustrating the structure of a MFE and the manufacturing steps thereof in another embodiment of the present invention.

FIGS. 7a to 7b are cross-sectional views illustrating the structure of a MFE and the manufacturing steps thereof in still another embodiment of the present invention.

#### DESCRIPTION OF THE PRESENTLY PREFERRED EMBODIMENTS

##### EXAMPLE 1

FIGS. 4a to 4d illustrate the method for manufacturing a MFE in this example.

FIG. 4a shows the state before forming the first anode and the emitter. Namely, an insulating layer 2 made of  $\text{SiO}_2$  film or  $\text{Al}_2\text{O}_3$  film was deposited on a conductive substrate 4 made of Si by the well known chemical vapor deposition method, thermal oxydization method or sputtering method to a thickness of 0.4 to 5  $\mu\text{m}$ , then a conductive layer 1 used for the first anode was deposited on the insulating layer 2 by the evaporation method. Next, as is shown in FIG. 4b, there was formed on the conductive layer 1 a photo-resist film 9 having a closed loop opening 14 of a predetermined pattern, at a predetermined position. The shape of the opening 14 was either circular or square when viewed from the topside, and the width,  $l_1$ , thereof was 0.3 to 3  $\mu\text{m}$ . The conductive layer 1 was exposed at the closed loop opening portion 14.

Next, the conductive layer 1 was etched employing the photo-resist film 9 with the opening 14 as a mask, and the insulating layer 2 was also etched employing the conductive layer 1 as a mask to thereby expose the substrate 4 at the closed loop opening portion 16. As is shown at FIG. 4c, there was formed on the conductive layer 1 a closed loop opening 15 with a width slightly broader than the width  $l_1$  of the opening 14 of the photo-resist film 9 and on the insulating layer 2 a closed loop opening 16, the cross-section of which had an inverse turncated conelike shape with an upper side slightly longer than the width of the opening 15.

Furthermore, a needlelike emitter with a sharp tip like that illustrated at FIG. 2d was formed under the islelike insulating layer 19 surrounded by the opening 16. Simultaneously, a minute cavity 18 was formed by sufficiently broadening the channel around the emitter 3 under the insulating layer 2, by etching the conductive substrate 4 employing the insulating layer 2 with the opening 16 of bottom side width  $l_2$  as a mask. The insulating layer 2 and the conductive layer 1 was made to overhang the minute cavity 18 of the substrate 4 by generating a large opening 16' in said insulating layer 19.

Finally, the resist film 9 was removed to thereby obtain a MFE according to the present invention, as illustrated in FIG. 4d.

As described above, it becomes possible to form a first anode 1 and an emitter 3 readily by only a series of etching steps. Since the emitter 3 was formed by the etching of the conductive substrate 4, there was no mixing of the mask material with the emitter as occurs in the previous method illustrated in FIGS. 3a to 3e. Therefore, electron emissions of high quality were obtained, and the manufacturing procedure could be simplified because of the lack of necessity of the removal of the mask material.

Furthermore, it becomes possible to remove many faults in the previous method as follows: there is no decrease of the dielectric breakdown voltage caused by contamination or the like because the insulating layer 2 disposed between the first anode 1 and the substrate 4 covers the lower surface of the first anode 1 and is so formed that it sufficiently overhangs the minute cavity 18 of the substrate 4 around the emitter 3.

## EXAMPLE 2

As illustrated in FIG. 5, a MFE was manufactured according to the same method as Example 1, then  $\text{LaB}_6$  particles 10 were vacuum-evaporated on the first anode 1 and the emitter 3 from a direction perpendicular to the surface of the substrate 4 to thereby form a first anode surface layer 11 and an emitter surface layer 12.

The resultant MFE had very good insulation between the substrate 4 and the first anode 1 because the insulating layer 2 made of  $\text{SiO}_2$  overhung by more than 1  $\mu\text{m}$  the minute cavity 18.

## EXAMPLE 3

FIGS. 6a to 6d illustrate the method for manufacturing a MFE in this example.

A  $\text{SiO}_2$  insulating layer 2 of about 2  $\mu\text{m}$  thickness was deposited on the substrate 4 made of a Si single crystal having a low specific resistivity, by the well known sputtering method, as shown at FIG. 6a. Then, a photo-resist film 9, which had a closed loop opening of a predetermined diameter and width at a predetermined position, was formed on the insulating layer 2. After that, the insulating layer 2 was etched, employing the photo-resist film 9 as a mask by the well known chemical etching method so as to form a closed circular loop opening 17 at a predetermined position in the surface of the insulating layer 2 thereby exposing the substrate 4 at the opening position 17 as illustrated in FIG. 6b. Next, the photo-resist film 9 was removed, and the substrate 4 was etched employing the etched insulating layer 2 as a mask by the well known chemical etching technique, thus forming a needlelike emitter with a sharp tip as shown at FIG. 6c. The islelike insulating layer 2" over the emitter 3 fell off at this time.

Finally,  $\text{LaB}_6$  particles 10 were vacuum-evaporated on the insulating layer 2 and the emitter 3 from a direction perpendicular to the surface of the substrate 4 as shown in FIG. 6d, thereby forming the first anode 11. An improvement in the electron emissivity of the emitter was achieved simultaneously by the activation of the surface 12 of the emitter 3 namely by lowering the work function thereof. Thus, the desired MFE was manufactured.

## EXAMPLE 4

A  $\text{LaB}_6$  layer 13 of about 10  $\mu\text{m}$  thickness was formed on a sapphire substrate 4 as illustrated at FIG. 7a. Then, an insulating layer 2 and a conductive layer 1 used for a first anode were deposited on the  $\text{LaB}_6$  layer 13. Next, the conductive layer 1, the insulating layer 2 and the composite substrate 20 were etched in this order by the same procedure as in Example 1 to form a needlelike emitter 3 and a cavity 18 over which the insulating layer 2 and the first anode layer 1 overhung. In this last step, the composite substrate 20 was so etched that the bottom of the cavity 18 around the emitter 3 did not reach the sapphire substrate 4. FIG. 7b illustrates the structure of the MFE thus manufactured.

## EXAMPLE 5

The properties of the MFE's of the present invention were compared with those of previous MFE's in this example.

The MFE of the present invention used in this example had the structure illustrated in FIG. 4d and had a Si

substrate 4 of 200  $\mu\text{m}$  thickness, an emitter 3 having a height of 2.5  $\mu\text{m}$  and a tip radius of curvature of 500  $\text{A}$ , a  $\text{SiO}_2$  insulating layer 2 of 2  $\mu\text{m}$  thickness and a first anode 1 of 0.5  $\mu\text{m}$  thickness made of Au. The previous MFE used in this example had the structure illustrated in FIG. 3e and had the same shape and thickness for each part as said MFE of the present invention, but it had no first conductive layer 5. Furthermore, both of the Si substrate faces had (111) crystalline planes. Mo was used for the emitter 3 and the first anode layer 1 of the previous MFE.

The atmospheres of these MFE's were made vacuum to  $1 \times 10^{-7}$  Torr, accelerating voltage of 200 V was applied between the emitters and the first anodes, and the emitted electron rays were further accelerated by a high applied voltage of 4 kV between the emitters and second anodes arranged over the emitters at 10 cm. distance.

As a result, the measured emission current density of the MFE of the present invention was about  $1 \times 10^5$   $\text{A}/\text{cm}^2$  which was 1.5 times that of the previous MFE which was about  $6 \times 10^4$   $\text{A}/\text{cm}^2$ . Furthermore, the stable working hours in which the emission current fluctuations were within  $\pm 5\%$  and wherein the intended emission currents were constantly 5  $\mu\text{A}$  were measured at about 500 hours for the MFE of the present invention and at about 250 hours for the previous MFE. Therefore, the life of the MFE of this invention was twice as long as the life of the previous MFE. Still further, the dielectric breakdown voltages between the first anode and the emitter were measured, and the resultant measured values for the MFE of this invention and for the previous MFE were about 1,000 V and about 500 V, respectively, wherein the thickness of the insulating layers was 2  $\mu\text{m}$ .

Desirable results were also obtained for MFE's having structures according to the other examples or drawings of this invention.

The reasons why MFE's having structures according to the present invention have superior properties are as follows:

1. Concerning the high dielectric breakdown voltage and the long life: the length of the surface of the insulating layer between the first anode 1 and the emitter 3 or the conductive substrate 4 is large, so that surface leakage and surface contamination during operation are minimal because the emitter side of the insulating layer 2 overhangs the minute cavity 18 as shown in FIG. 4d.

2. Concerning the long life: there occurs no inferiority at the portion where the emitter 3 is connected with the conductive substrate thereunder, because the emitter 3 and the conductive substrate 4 are comprised as one body.

3. Concerning the high emission current density: the upwards gradient of the electric field at the tip of the emitter is sharp under the application of voltage between the electrodes, because the tip of the emitter 3 is never higher than the bottom level of the first anode 1.

While the novel principles of the invention have been described, it will be understood that various omissions, modifications and changes in these principles may be made by one skilled in the art without departing from the spirit and scope of the invention.

What is claimed is:

1. A thin-film field-emission electron source comprising a conductive substrate having a minute cavity, a needlelike emitter within said cavity, an insulating layer

on the surface of said substrate except for the portion of said cavity, and a first anode layer on said insulating layer, wherein said emitter and said substrate are formed as a single body, and said insulating layer and said first anode layer overhang said cavity around the projection of said emitter except over said emitter.

2. The thin-film field-emission electron source of claim 1, in which said substrate is composed of an insulating plate and a conductive layer formed on said insulating plate.

3. The thin-film field-emission electron source of claim 1, in which said substrate is made of a material selected from the group consisting of Si, W, W alloyed with Th, and Mo.

4. The thin-film field-emission electron source of claim 1, in which said insulating layer is made of a material selected from the group consisting of  $\text{SiO}_2$ ,  $\text{TiO}_2$ ,  $\text{Ta}_2\text{O}_5$ ,  $\text{Y}_2\text{O}_3$ ,  $\text{Si}_3\text{N}_4$ , AlN, alumina and heat resisting glass.

5. The thin-film field-emission electron source of claim 1, in which the surface of said emitter is coated with a material selected from the group consisting of  $(\text{Ba},\text{Sr})\text{O}$ ,  $(\text{BaO}-\text{SrO}-\text{CaO})$ ,  $(\text{Ca},\text{Sr})\text{O}$ ,  $\text{LaB}_6$ ,  $\text{CaB}_6$ ,  $\text{SrB}_6$ ,  $\text{BaB}_6$ ,  $\text{CeB}_6$ ,  $(\text{La},\text{Sr})\text{B}_6$ ,  $(\text{La},\text{Ba})\text{B}_6$ ,  $(\text{La},\text{Eu})\text{B}_6$ ,  $(\text{Ce},\text{Sr})\text{B}_6$ ,  $(\text{Ce},\text{Ba})\text{B}_6$ ,  $(\text{Ce},\text{Eu})\text{B}_6$ ,  $(\text{Pr},\text{Sr})\text{B}_6$ ,  $(\text{Pr},\text{Ba})\text{B}_6$ ,  $(\text{Pr},\text{Eu})\text{B}_6$ ,  $(\text{Nd},\text{Sr})\text{B}_6$ ,  $(\text{Nd},\text{Ba})\text{B}_6$ ,  $(\text{Nd},\text{Eu})\text{B}_6$ ,  $(\text{Eu},\text{Sr})\text{B}_6$  and  $(\text{Eu},\text{Ba})\text{B}_6$ .

6. The thin-film field-emission electron source of claim 1, in which said first anode layer is made of a material selected from the group consisting of Cr, Au, Ni and their alloys.

7. The thin-film field-emission electron source of claim 5, in which the first anode layer is made of the same material as said surface of said coated emitter.

8. The method for manufacturing the thin-film field-emission electron source according to claim 1, comprising the steps: i) forming an insulating layer on a conductive substrate, ii) forming a first anode layer made of a conductive material on said insulating layer, iii) forming an annular opening at a predetermined position on said first anode layer by etching, iv) form-

ing an annular opening on the face of said insulating layer under the opening provided in step iii) by etching said insulating layer employing said first anode layer as a mask, and v) forming a minute cavity and a needlelike emitter on said substrate by etching said substrate employing said insulating layer as a mask.

9. The method of claim 8, in which said insulating layer is formed by a chemical vapor deposition method.

10. The method of claim 8, in which said insulating layer is formed by a thermal oxydization method.

11. The method of claim 8, in which said insulating layer is formed by a sputtering method.

12. The method of claim 8, in which said first anode layer is formed by an evaporation method.

13. The method of claim 8, in which said etchings of steps iii), iv) and/or v) are carried out by chemical etching.

14. The method of claim 8, in which said etchings of steps iii), iv) and/or v) are carried out by physical etching.

15. The method of claim 8, further comprising a step of depositing an electron emissive material layer on said emitter after said step v).

16. A method for manufacturing the thin-film field-emission electron source according to claim 1, comprising the steps: i) forming an insulating layer on a conductive substrate, ii) forming an annular opening at a predetermined position on said insulating layer by etching, iii) forming a minute cavity and a needlelike emitter on said substrate by etching said substrate employing said insulating layer as a mask, and iv) depositing an electron emissive material layer on said insulating layer and said emitter.

17. The thin-film field-emission electron source of claim 1, in which the numbers of said cavities, said emitters and said first anode layers are plural.

18. The thin-film field-emission electron source of claim 1, in which the overhang of said insulating layer over said cavity is greater than  $0.5 \mu\text{m}$ .

19. The thin-film field-emission electron source of claim 18, in which said overhang is greater than  $1 \mu\text{m}$ .

\* \* \* \* \*